

## UNITED STATES PATENT OFFICE.

CARL HERMANN VON HOESSLE AND WALTER RICHTER, OF RADEBEUL, NEAR DRESDEN, GERMANY, ASSIGNORS TO CHEMISCHE FABRIK VON HEYDEN, OF RADEBEUL-DRESDEN, GERMANY, A CORPORATION OF GERMANY.

## FOIL FOR ORNAMENTING AND PRINTING PURPOSES.

No Drawing.

Application filed August 26, 1926. Serial No. 131,968.

This invention relates to transfer sheets and it particularly relates to transfer sheets consisting of a foil made for ornamenting and printing purposes.

5 Foils for printing, blocking and embossing are generally very brittle and many difficulties arise in using same. More solid foils are obtained by spreading a layer of colour or bronze-powder mixed with an adhesive mate-  
 10 rial on a suitably prepared paper, especially on so-called pergamyn-paper. By the action of the die, the coloured mass separates from the paper and remains on the printed subjects whereas the paper is taken away. It is a  
 15 disadvantage of this method that the structure of the paper, which had served as a vehicle for the colour, often injures the lustre of the prints and ornaments. According to a process of which one of the applicants, Hermann v. Hoessle, is the inventor, and which is described by the German Letters-Patent 368,274 a much better printing-foil is obtained by using instead of paper as a vehicle for the colour, a film of a cellulose-ester or of  
 20 25 hydrated cellulose, so-called cellophane. More brilliant prints are thus obtained owing to the smooth surface of such films and this process is satisfactory in almost all its aspects. A draw-back of these printing films is  
 30 that it is rather difficult to spread the pigment mixture in a uniform layer upon the smooth surface of the cellulose-film. This unevenness in the thickness of the colored mixture on the film is offering difficulties in so far  
 35 as an occasionally somewhat thicker layer of colored mass fills the die with an excess of material which subsequently is more heavily pressed by the die than a thinner layer, the result being that the prints often are defective as the coloured mass in such a case then does not readily separate from the film.

Now we have found that we can make a much better transfer sheet for printing or ornamenting purposes if we coat a foil or film  
 40 made of a smooth, flexible and preferably transparent organic matter, for instance a film of cellulose, a cellulose ester, gelatine, or similar material having inherently polished, glass-like surfaces, with a fine and even coat  
 45 of a mixture of wax, resin or similar glutinous

substance and of a layer of color or bronze in the form of a powder, both layers being homogeneously blended, without any mechanical agitation of the same, on the film. This blending takes place owing to the difference in the specific gravity of the materials of the layers blended together. Our new transfer sheet is made by applying to the film first a layer of wax, resins or other glutinous substances by spreading upon the film a solution of such adhesive, wax-like bodies in organic solvents, or by distributing the wax or resins in melted condition on the film by brushes or rollers.

A second layer of color or bronze powder is now produced on and mixed with the first one. The color or bronze powder may be evenly sprayed on either when suspended in a solution of resins or other resinous material in benzene, alcohol, or any other suitable organic solvent, or in the form of a dry powder. The adhesive power of the first layer of wax or the like is brought out by treating it with an organic solvent and as the first layer is thus re-dissolved, the aforesaid solution carrying the heavy powder of color or bronze, mingles with the solution of the first layer, so that the powder of color or bronze becomes embedded therein when the layer becomes dry. In the other case, when the powder of color or bronze is sprayed on in dry form, the film with the first layer is slightly heated and the wax or resin, being melted the surface of the film, is then treated with the powder of color or bronze, which sinks into the molten wax or the like so as to be thoroughly and evenly mixed with the same when it becomes solid again. Thereupon a third layer, consisting of a solution of shellac, colophonium, artificial resins, bakelite or the like may be applied. Prints made with such printing films are very durable. It is not necessary any more to treat the surfaces on which the impression shall be made with an adhesive material before printing.

The die may be cold or warm. No more brushing away of portions which do not belong to the design is necessary. The impression obtained is very sharp, for as soon as the pressure of the die has ceased, the film can be

removed together with all those parts of its layer, which have not been used up in the printing.

The following examples will illustrate the process described above.

*Example 1.*

80 parts by weight of carnauba-wax, 20 parts by weight of colophonium and 10 parts 10 by weight of bees-wax are dissolved in 700 parts of hot toluene. The solution is finely distributed upon a film of cellulose (cellophane). That is effected by passing the film over a rotating roll dipping into a trough 15 containing said solution, which is heated to about 70 degrees centigrade. The film then passes a heated cylinder until absolutely dry.

In order to give the film a second or middle 20 layer, it must pass a box with a rotating cylinder, which is heated to about the melting-point of the wax. The box contains bronze-powder. On its way along the box, the film, 25 with its cellophane-side, touches the cylinder, whereas the wax-side begins to melt and gets coated with a layer of the bronze-powder. An excess of the latter is removed by rotating brushes after the film has cooled off. A third layer is now put on the film by running 30 it over a roll covered with felt which gets continuously soaked with a 15 per cent solution of shellac in alcohol. The film is again dried by a hot rotating cylinder.

*Example 2.*

35 A cellophane-film covered with a first layer of wax is treated in a dipping-apparatus with a solution of 20 parts by weight of colophonium in 60 parts of ethyl alcohol, 30 parts of ether and 30 parts of benzene which has been 40 well mixed with 100 parts by weight of a red

mineral colour. The film is then dried on a hot cylinder. No third layer of shellac is necessary in this case.

Now what we claim is:

1. In a transfer sheet the combination comprising a carrier film of an inherently smooth and non-porous structure-less material, a layer of a mass having a low melting point and a moderate adhesive power, a middle layer of coloring matter each particle of which is encased in a binding material, and a top layer of a mass melting at a relatively higher temperature and having an adhesive power greater than the other fusible mass referred to above. 55

2. In a transfer sheet the combination comprising a carrier film of an inherently smooth non-porous structure-less material, a layer of a mass having a low melting point and a moderate adhesive power, a middle layer of 60 coloring matter each particle of which is encased in a binding material melting at a relatively higher temperature and having an adhesive power relatively greater than that of the aforesaid layer, and a top layer of a material substantially identical with that of the aforesaid middle layer. 65

3. In a transfer sheet the combination comprising a carrier film of an inherently smooth non-porous structure-less material, a layer 70 consisting chiefly of a mixture of waxes and to a minor part of colophonium, a middle layer of coloring matter and a top layer of rosins of relatively great adhesive power, encasing the particles of the middle layer. 75

In testimony whereof we have affixed our signatures.

CARL HERMANN von HOESSLE.  
WALTER RICHTER.